

## UNITED STATES PATENT OFFICE

CAMILLE DREYFUS, OF NEW YORK, N. Y., GEORGE W. MILES, OF BOSTON, MASSACHUSETTS, AND HERBERT PLATT, OF CUMBERLAND, MARYLAND, ASSIGNEES TO CELANESE CORPORATION OF AMERICA, A CORPORATION OF DELAWARE

## COLORING OF TEXTILE MATERIALS

No Drawing.

Application filed February 25, 1929. Serial No. 342,667.

This invention relates to the coloring of textile materials such as fabric or yarn and relates more particularly to the coloring of such material by means of water insoluble colloidally dispersed coloring matter.

An object of our invention is to impart a light-fast color to textile materials by treating the same with a substance containing a colloidally dispersed water insoluble coloring matter, such as mineral pigments and/or water insoluble organic dyestuffs. A further object of our invention is to decrease the tendency of coloring matter to rub off from textile material by the incorporation in the substance containing the coloring material of latex or colloidal rubber. A further object of our invention is to diminish the tendency of fabrics to slip or ladder by treating the same with a suspension of latex. Further objects of our invention will appear from the following detailed description.

We have found that if textile materials, and particularly textile materials containing organic derivatives of cellulose, are treated with colloidal suspensions or solutions of mineral pigments, these pigments are absorbed by the textile material, whereby color effects which are extremely fast to light are obtained. In order to prevent or diminish the tendency of the coloring matter to rub off, we have found that the addition to the substance containing the same of colloidal rubber or latex is advantageous. Moreover if such fabrics are treated with a suspension of latex, the tendency of the same to run or ladder is reduced.

In accordance with our invention, we treat textile materials with a substance containing a finely divided mineral pigment and/or water soluble or insoluble organic dyestuff in colloidal suspension or solution, and preferably but not necessarily in the presence of colloidally dispersed rubber or latex.

The textile material to be treated in accordance with our invention may be yarn or fabric. The yarn may be treated in the form of hanks or wound onto suitable packages such as bobbins, pirns, cones, etc. The fabric may be any suitable woven, knitted or netted fabric.

While this invention is of general application and is applicable to textile materials made of all kinds of fibres, it is of special interest in the coloring of yarns containing organic derivatives of cellulose or fabrics consisting in whole or in part of such yarns. The organic derivatives of cellulose may be organic esters of cellulose or cellulose ethers. Examples of organic esters of cellulose are cellulose acetate, cellulose formate, cellulose propionate and cellulose butyrate, while examples of cellulose ethers are ethyl cellulose, methyl cellulose and benzyl cellulose.

The fabric may be a mixed fabric containing yarns of such organic derivatives of cellulose and yarns of other fibres such as cotton, natural silk, wool, reconstituted cellulose (rayon) etc.

Any suitable mineral pigment may be employed in our invention. Examples of such pigments are graphite, prussian blue, vermillion, red lead, or other suitable pigments that are employed in the making of paints. If desired, organic dyestuffs such as ponsol blue 3-G, anthrene jade green, other vat colors, the azo dyestuffs or other water soluble dyestuffs may also be employed, and any suitable mixtures of the mineral pigments and/or water soluble or insoluble organic dyestuffs to obtain the desired color are applicable. In order to cause the textile materials to become colored, it is of importance that the pigments and/or water insoluble dyestuffs be applied thereto preferably in the form of a colloidal dispersion or solution, or in such fine degree of dispersion as will produce the desired coloration.

In order to reduce the tendency of the coloring material to rub off of the textile material after the same has been colored therewith, we prefer to add to the dye bath or printing paste containing such coloring material an appropriate amount of colloidal rubber or latex to which a suitable vulcanizing agent may be added if desired. The textile material may if desired be treated with a bath containing latex and no coloring matter, and this treatment may be carried out on the undyed fabric or yarn, or on such fabric or yarn after the same has been dyed.

In order to increase the affinity of the textile material for the pigment, we prefer to add to the dye bath or printing paste, suitable substances that act as assistants for causing

- the textile material to have the color imparted thereto. These assistants may be in the form of swelling agents for the fibers of the textile material and/or in the form of inorganic or organic salts such as sodium chloride, sodium or potassium hydrosulphite, the thiocyanate of ammonium, potassium or sodium, or other salts of a strong base and a weak acid, such as borax. In some cases organic compounds which may also act as swelling agents for the organic derivatives of cellulose in the textile material may be employed and examples of these are acetic acid, formic acid, acetone, etc.

Due consideration should be given to the nature of the substances employed as assistants to promote the coloring of the textile material and the concentration of the same employed. Thus if no latex is employed, we have found that the use of sodium chloride in

- amounts from 2 to 20 grams per liter of dye bath give highly satisfactory results. When latex is employed in conjunction with the colloidal pigment or water insoluble dye-stuff, the salts of a strong base and weak acid, such as ammonium thiocyanate or borax, are very advantageously employed, and their concentration should be such that the coagulation of the latex is avoided. Thus in the case of ammonium thiocyanate, a concentration of from 0.5 to 2 grams per liter or more produce satisfactory results. Since acids cause the coagulation of latex, if the textile material is to be dyed with a dye that requires the presence of acid, this dyeing is preferably done prior to treatment with the bath containing the latex.

In the case of a mineral pigment such as colloidally dispersed graphite, the use of the hydrosulphite of sodium or potassium is quite feasible, and since these hydrosulphites are often employed in connection with the vat dyes, this invention may be employed for shading the colors obtained by dyeing textile materials with such vat dyes. Thus by incorporating a suitable amount of colloidal graphite in a dye bath or printing paste containing a vat dye, and an alkaline hydrosulphite the color imparted to the textile material by such bath or paste may be deepened or darkened or shaded to any desired degree. This shading effect may be obtained in connection with any suitable dyestuff.

This invention may be employed for dyeing textile materials by immersing the same in a dye bath made in accordance with this invention. Moreover local color effects may be produced by printing with a suitable paste containing a suitable thickening agent such as gum arabic, gum tragacanth or British gum and the colloidally dispersed coloring

material. Also by brushing or spraying a solution made in accordance with our invention through stencils onto fabrics, differential color effects may be obtained.

In order further to illustrate our invention but without being limited thereto the following specific examples are given.

#### Example I

The following is an example of the treatment of a fabric with an aqueous bath containing latex.

A fabric consisting wholly of cellulose acetate yarn is worked in a bath for one hour at 75° C., which bath contains 25 cc. per litre of latex (30%) and 5 grams per litre of ammonium thiocyanate. If the fabric so treated is a woven fabric, the tendency of the same to slip is considerably less than that of an untreated fabric, whereas if the fabric is a knit fabric its tendency to ladder is materially reduced.

#### Example II

A fabric consisting wholly of yarns of cellulose acetate is treated in a bath containing 5 grams per liter of sodium chloride and 10% of an aqueous colloidal dispersion of graphite. The time of treatment is  $\frac{3}{4}$  of an hour and the temperature is 75° C. The fabric has a medium gray color imparted thereto, which color is fairly fast to washing and which is extremely fast to light. If instead of employing 10% of the dispersion of graphite, 40% thereof is employed, a very dark gray color is imparted to the fabric, which color has a good fastness to washing and a very good fastness to light.

#### Example III

The following is an example wherein colloidal rubber or latex is employed to prevent or diminish the tendency of the color to rub.

A fabric consisting wholly of yarns of cellulose acetate is treated for  $\frac{3}{4}$  of an hour at 75° C. in 50 times its weight of a bath which is made up as follows:

Aqueous colloidal dispersion of graphite 10% 115  
Ammonium thiocyanate 1 gram per liter  
Latex (30%) 5 cc. per liter

A medium gray color is imparted to the fabric, which color is fast to washing, very fast to light and which color does not rub.

If instead of employing 10% of graphite, 40% of the same is used, a dark gray color that is fast to washing, light and rubbing is obtained.

It is to be understood that the foregoing detailed description is given merely by way of illustration and that many variations may be made therein without departing from the spirit of our invention.

Having described our invention what we

claim and desire to secure by Letters Patent is:

1. Textile material containing cellulose acetate having a color imparted to at least 5 part of the surface thereof by means of a dispersion of finely divided graphite.
2. Textile material containing cellulose acetate having a color imparted to at least part of the surface thereof by means of finely 10 dispersed graphite and latex.
3. Method of coloring textile materials containing organic derivatives of cellulose, comprising applying thereto by means of a bath treatment a dispersion of finely divided graphite. 15
4. Method of coloring textile materials containing cellulose acetate, comprising applying thereto by means of a bath treatment a dispersion of finely divided graphite.
5. Method of coloring textile materials containing organic derivatives of cellulose, comprising applying thereto by means of a bath treatment a dispersion of finely divided graphite in the presence of a substance that 20 acts as an assistant for imparting color.
6. Method of coloring textile materials containing cellulose acetate, comprising applying thereto by means of a bath treatment a dilute colloidal dispersion of latex and a dispersion of finely divided graphite. 25
7. Method of coloring textile materials containing cellulose acetate, comprising applying thereto by means of a bath treatment a dilute colloidal dispersion of latex and a dispersion of finely divided graphite in the presence of a substance that acts as an assistant for imparting the color.

In testimony whereof, we have hereunto subscribed our names.

40 CAMILLE DREYFUS.  
GEORGE W. MILES.  
HERBERT PLATT.

45

50

55

50

35